

## UNITED STATES PATENT OFFICE

2,232,460

## DYEING UNION FABRICS CONTAINING POLYVINYL HALIDE-ACETATE COPOLYMERS

Arthur Frederick Klein, Philadelphia, Pa., assignor to American Cyanamid Company, New York, N. Y., a corporation of Maine

No Drawing. Application December 23, 1939,  
Serial No. 310,834

8 Claims. (Cl. 8—21)

This invention relates to the dyeing of union goods containing polyvinyl halide-acetate copolymer fibers.

The dyeing of polyvinyl halide-acetate copolymer material which has been put on the market under the trade name of "Vinyon" has presented a considerable dyeing problem. Not only is the material difficult to dye and has required the use of such auxiliary measures as the employment of solvents for the material in the dye bath, or as described in the copending application of Kienle and Petke, Ser. No. 309,608, filed December 16, 1939, the use of assistants of the amine, phenol, ester and open chain ether type, but the material has been found to be very heat sensitive. If the temperature of the bath is not kept below a certain figure, a very serious shrinkage of the "Vinyon" takes place.

This property of shrinking has been practically utilized in the manufacture of union felt materials to be felted containing a mixture of "Vinyon" and other fibers. It has been suggested to hot press the material at a temperature sufficiently high to cause substantial shrinking of the "Vinyon." This shrinking increases the strength and wearing ability of the felt as the shrunk "Vinyon" fibers appear to anchor with the other fibers in the felt and hence to produce a stronger and if desired, thinner product. Attempts have been made to dye such felts following the general practice of low temperature dyeing and dyed felts can be produced by this procedure in two steps, the felt being first hot shrunk and then cold dyed.

The present invention produces similar advantageous results in a single step in felts and other union materials containing "Vinyon" fibers. Instead of hot shrinking the material, and then cold dyeing, I have found that if the dye bath is maintained at a sufficiently high temperature, for example, above 75° C., the union goods are dyed and the "Vinyon" shrunk in a single operation and level dyeing is achieved with uniform shrinkage. Not only is it possible to obtain good results in a single step by the present invention which required two steps before, but the dyeing procedure is actually improved because the high temperature permits more rapid and efficient dyeing not only of the "Vinyon" but of many of the other fibers which may be associated therewith. Material savings in time and improved results are therefore obtained.

The present invention is applicable not only to union felts, but also to other union fabrics where shrinkage of the "Vinyon" component is of importance. Thus colored crepe fabrics and other fancy effects may be produced by a single step process by means of the present invention and in every case improved results are obtained.

It is an advantage of the present invention

that the ordinary procedures in union dyeing need not be materially changed over standard dyeing procedures, except of course, that the dye bath must contain the necessary ingredients for dyeing "Vinyon" if it is to be colored. In certain cases the dye bath is deliberately so chosen that it will not dye the "Vinyon" but it will dye the other fibers producing goods with white stripes or other effects.

The present invention is not critical as to temperature and in general temperatures above 75° C. may be used. Shrinkage begins at about this temperature and rapidly increases. At temperatures of about 100° C. the shrinkage is very marked and operation at this temperature has the advantage that it is easy to maintain a uniform temperature if the dye bath is permitted to boil gently. Still higher temperatures may of course be used and suitable dyeing under pressure can be employed but care should be taken that the temperatures do not approach that at which the polyvinyl halide-acetate copolymer begins to soften as otherwise the fibers may be damaged. In general this upper limit is about 135° C. and should not be approached too closely unless the surface changes in the "Vinyon" which take place are unobjectionable.

The proportion of "Vinyon" in the mixed goods or union fabrics may vary within wide limits. The present invention is not being limited to any particular proportion. In general the amount of "Vinyon" used will be sufficient to produce the desired result. Where it is mixed with cheaper fibers such as cotton, rayon, and the like, it is generally economically desirable to keep the proportion of "Vinyon" down as low as possible and consistent with obtaining the effect desired. It is an important advantage of the present invention that in many cases even small amounts of "Vinyon" will produce remarkable results when high temperature uniform dyeing is employed.

The present invention is not limited to the use of any particular dyes or any particular mixture of dyes. The dyeing procedures form no part of the present invention except insofar as they have to be modified to effect high temperature dyeing. It is an important advantage of the present invention that at the high dyeing temperatures used, it is not necessary to employ either solvent or non-solvent dyeing assistants as the high temperature apparently affects the surface of the "Vinyon" so that it will accept suitable oil soluble dyes. Not only does the present invention produce improved results but the dyeing procedure is actually simplified and the cost of solvents or non-solvent assistants can be saved.

When vat or sulfur dyeing is desired it is advantageous to use the specific procedures disclosed and claimed in the copending application

of Petke and Klein, Ser. No. 310,828, filed December 23, 1939.

The invention will be described in greater detail in conjunction with the dyeing of typical mixed or union material in the following specific examples, it being understood that the invention is not limited to the details therein set forth.

*Example 1*

10 100 parts of a felt containing 72% cotton, 7% wool and 21% "Vinyon" is dyed in the following manner: 3.02 of a dry blend of water dispersible color which contains 2.2 parts of benzopurpurine (C. I. 448), 0.02 part of a direct dyeing blue (C. I. 518), and 0.80 part of an oil-soluble color made by coupling p-nitroaniline on phenyl ethyl ethanolamine is stirred into 3000 parts of water. 30 parts of salt is added and 1/2 part of dioctyl sodium sulfosuccinate is added. The felt which is wet out with dioctyl sodium sulfosuccinate is entered into the cold bath. The temperature of the dyebath is raised during a period of 20 minutes to the boil, the dyeing is continued for 20 minutes at the boil, and for 20 minutes longer in the cooling bath. The dyed felt is rinsed and dried. The material is dyed a bright red which is level and does not crock or sublime.

*Example 2*

30 100 parts of a knit fabric composed of 75% rayon and 25% "Vinyon" is dyed in the following manner: 2.31 parts of a dry blend of dispersed and soluble colors, containing 1.5 parts of a direct dyeing color (C. I. 518), 0.07 part of a direct dyeing green (Pr. 693), 0.60 part of dispersed 1-methyl amino-4-ethylol amino anthraquinone, and 0.04 part of a dispersed oil-soluble orange made by coupling diazotized p-nitroaniline on p-xylidine, are stirred into 3000 parts of water. 30 parts of common salt and 0.5 part dioctyl sodium sulfosuccinate are then added and the fabric which has been wet out is placed in the bath. The temperature of the bath is raised to 150° F., held at this temperature for 30 minutes, and then raised to the boil and held there for 30 minutes. The dyed fabric is then rinsed and dried. This procedure gives a fabric in which the two fibers are dyed the same shade and strength and which does not crock or sublime.

*Example 3*

5 parts of a union fabric composed of 30 parts of "Vinyon" and 70 parts of wool are dyed with 55 a bath prepared in the following manner: 0.1 part of a Red Vat color (Pr. 89) is reduced with 1 part of a 60% solution of ethylene diamine and 1 part of sodium hydrosulfite. 0.5 part of dibutyl phthalate and 0.3 part of a 10% solution of ammonium linoleate are added, followed by stirring, to give a smooth paste. This paste is then diluted with 150 parts of water and the fabric dyed therein for 1 hour at 85° C. Under these conditions the color exhausts well from the bath. The 65 dyed cloth is then oxidized with any of the usual oxidizing agents, soaped and dried. This procedure gives a level, red union dyeing with good fastness properties.

The specific examples refer to the use of wet 70 out fabric or yarn. This is a desirable procedure and very effective results can be obtained by the use of dilute solutions of powerful wetting agents such as for example a 1/2% solution of dioctyl sodium sulfosuccinate. The invention is however 75 not limited to pre-wetting material where the

nature of the material is such that satisfactory dyeing can be obtained with unwet material.

The examples all show the dyeing at high temperatures of union materials in which the "Vinyon" fibers are unshrunken so that the dyeing procedure performs at the same time coloring and all of the shrinking of the "Vinyon" which is to take place. For many types of goods this is the most advantageous method because all the functions of shrinking and coloring are performed in 10 a single step with a minimum cost for equipment and labor. This constitutes the preferred embodiment of the invention. However, it should be understood that the invention is also of importance where for convenience in handling or 15 other reasons the union material has been subjected to a heat treatment, such as for example hot pressing of felt, which has resulted in partial shrinkage of the "Vinyon" fibers. In such a case the present invention still retains the important 20 advantage of rapid dyeing and good penetration which results from the high temperature bath, but most of the shrinkage may have been effected in a single step. In a broader aspect therefore, the invention includes dyeing at high tempera- 25 ture, union material which may have been partially pre-shrunk.

What I claim is:

1. A method of dyeing mixed materials containing substantially unshrunken polyvinyl halide- 30 acetate copolymer fibers admixed with other fibers which comprises subjecting the mixed material to dyeing in a dyebath at a temperature at which the unshrunken polyvinyl halide-acetate copolymer fibers show marked shrinkage. 35

2. A method of dyeing mixed materials containing substantially unshrunken polyvinyl halide-acetate copolymer fibers admixed with other fibers which comprises subjecting the mixed material to dyeing in a dyebath at temperatures 40 about 100° C.

3. A combined method of dyeing and increasing the strength of felts containing substantially unshrunken polyvinyl halide-acetate copolymer fibers admixed with other fibers which comprises dye- 45 ing the felt in a dyebath at a temperature at which the unshrunken polyvinyl halide-acetate copolymer fibers show marked shrinkage.

4. A combined method of dyeing and increasing the strength of felts containing substantially un- 50 shrunken polyvinyl halide-acetate copolymer fibers admixed with other fibers which comprises dyeing the felt in a dyebath at temperatures about 100° C.

5. A method according to claim 1 in which the 55 dyebath contains oil-soluble dyes and is substantially free from solvents for the polyvinyl halide-acetate copolymer and non-solvent dye assistants therefor.

6. A method according to claim 2 in which the 60 dyebath contains oil-soluble dyes and is substantially free from solvents for the polyvinyl halide-acetate copolymer and non-solvent dye assistants therefor.

7. A method according to claim 3 in which the 65 dyebath contains oil-soluble dyes and is substantially free from solvents for the polyvinyl halide-acetate copolymer and non-solvent dye assistants therefor.

8. A method according to claim 4 in which the 70 dyebath contains oil-soluble dyes and is substantially free from solvents for the polyvinyl halide-acetate copolymer and non-solvent dye assistants therefor.